

## UNITED STATES PATENT OFFICE

ROBERT T. WOOD, OF LAKWOOD, OHIO, ASSIGNOR, BY MESNE ASSIGNMENTS, TO  
MAGNESIUM DEVELOPMENT CORPORATION, A CORPORATION OF DELAWARE

## MAGNESIUM BASE ALLOYS

No Drawing.

Application filed May 19, 1931. Serial No. 538,607.

The invention relates to magnesium base alloys. Heretofore, these alloys have contained as essential alloying elements such metals as aluminum, copper, and cadmium. So far as I am aware, no one has heretofore produced or investigated alloys containing magnesium in large amount and smaller, but effective, amounts of zinc, tin, and calcium, in which manganese may also be a valuable alloying element.

I have discovered that magnesium base alloys containing tin, zinc, and calcium with or without manganese may be cast, rolled, forged, extruded, and similarly treated according to well known methods, provided the proper proportions of each alloying element be present as hereinafter disclosed. They are also susceptible of improvement by the ordinary heat treatments known to the art, and in addition, the physical properties, especially the yield point and hardness, of these alloys may be substantially improved by so-called "artificial aging" treatment subsequent to the usual elevated temperature heat treatments. I have discovered that useful alloys of this nature may be compounded containing from about 0.1 per cent to about 20 per cent tin, from about 0.1 per cent to about 10 per cent zinc, and from about 0.05 per cent to about 2.0 per cent calcium. If manganese be added in amount from about 0.1 per cent to about 2.5 per cent, the hardness and other beneficial properties of the alloy are also increased.

The particular composition of each constituent to be chosen depends upon the use to which the alloy is to be put. Considering, for instance, the constituent zinc, if the alloy be intended for casting purposes, an amount of from about 2 per cent to about 6 per cent is suitable, and I prefer to use about 4 per cent, whereas for purposes of extrusion from about 0.1 per cent to about 10 per cent of zinc may be advantageously added to the alloy. If an alloy for forging or rolling is desired, the zinc is preferably present in amount not less than about 0.1 per cent and not greater than about 1.0 per cent.

The element tin may be incorporated in the alloy in amounts from about 4 per cent to about 8 per cent for casting purposes, and for forgings or for extrusion purposes in amounts from about 0.1 per cent to about 20.0 per cent, although I prefer to add tin in amounts between 4 per cent and 12 per cent.

The element calcium should, for casting purposes, be preferably kept below about 0.5 per cent but may be used in amounts from about 0.1 per cent to 2 per cent in forged or extruded products.

If the element manganese be added as a hardener, it should, in casting alloys, be preferably lower than 1 per cent, although from 0.1 per cent to about 2.5 per cent can be used in alloys to be forged or extruded.

My new alloys may be made up according to the usual metallurgical methods of alloying but I prefer to add the tin and manganese to the molten magnesium in the form of an alloy of tin and manganese suitably proportioned in metal content to give the desired final ratio of tin and zinc in the alloys. The calcium may be added in the form of pure calcium. The zinc may be added either separately or as a tin-zinc rich alloy. The magnesium, tin, zinc, calcium, and manganese from which the alloys are made may or may not contain impurities, depending upon the purity of the metal available, but in any event small amounts of impurities even up to about 1 per cent may be present in the alloys without seriously affecting their favorable mechanical properties. Such alloys as are herein disclosed also have a high resistance to corrosion in comparison with magnesium base alloys hitherto commercially available.

As an illustration of the increase in yield point to which alloys within the scope of my invention are inherently susceptible, I have made up an alloy containing about 5 per cent tin, about 3 per cent zinc, about 0.73 per cent manganese, and about 0.25 per cent calcium and cast test specimens in sand molds. After casting, the yield point was 8,800 pounds per square inch, the tensile strength 23,900 pounds per square inch, and

the Brinell hardness 44. After a solution treatment of 24 hours at 500° centigrade followed by an aging treatment of 24 hours at 150° centigrade, the yield point was 5 18,200 pounds per square inch, the tensile strength 31,900 pounds per square inch, and the Brinell hardness 56.

An increase in yield point similarly phenomenal in nature, although numerically not

- 10 so great, is observable if the alloys be artificially aged after casting and without preliminary heat treatment at an elevated temperature. For instance, a sand cast alloy containing 5.4 per cent tin, 4.55 per cent 15 zinc, 0.72 per cent manganese, and 0.25 per cent calcium in the as-cast condition had a yield point of 9,910 pounds per square inch and a Brinell hardness of 44, and after an 20 artificial aging of 24 hours at 150° centigrade, it had a yield point of 14,550 pounds per square inch and a hardness of 57.

A sand cast magnesium base alloy containing about 5 per cent tin, 5 per cent zinc, and 0.25 per cent calcium was tested in the 25 as-cast condition and had a yield point of 10,200 pounds per square inch, a tensile strength of 22,600 pounds per square inch, an elongation of 4.7 per cent in 2 inches, and a Brinell hardness of 46.

- 30 A sand cast magnesium base alloy containing about 5 per cent tin, about 4 per cent zinc, and about 0.25 per cent calcium in the as-cast condition had a yield point of 9,450 pounds per square inch, a tensile 35 strength of 22,640 pounds per square inch, an elongation of 5.5 per cent in 2 inches, and a Brinell hardness of 45. After a heat treatment of 24 hours at 550° centigrade, it had a yield point of 9,050 pounds per square 40 inch, a tensile strength of 29,080 pounds per square inch, an elongation of 9.2 per cent in 2 inches, and a Brinell hardness of 45. Specimens thus heat treated were, in addition, aged 24 hours at 150° centigrade and 45 had a yield point of 19,240 pounds per square inch, a tensile strength of 32,230 pounds per square inch, an elongation of 3.7 per cent in 2 inches, and a Brinell hardness of 59. On heat treatment and artificial aging, there is apparent an increase in 50 yield point of almost 10,000 pounds per square inch, an increase in strength of almost 10,000 pounds per square inch, and an increase in hardness of over 14 Brinell numbers.

In the worked condition, alloys within the scope of this invention have exceptionally good physical properties. For instance, an extruded magnesium base alloy containing about 4 per cent tin, 3 per cent zinc, 0.2 per cent calcium, and 2.5 per cent manganese had a yield point of 26,000 pounds per square inch, a tensile strength of 46,000 pounds per square inch, and an elongation of 13.5 per cent in 2 inches. Similarly, an

extruded magnesium base alloy containing about 8 per cent tin, 3 per cent zinc, 0.2 per cent calcium, and 1 per cent manganese had a yield point of about 27,300 pounds per square inch, a tensile strength of about 45,000 pounds per square inch, an elongation of 10 per cent in 2 inches, and a Brinell hardness of 66.

The heat treatment which I have found especially suited to these alloys consists in a preliminary treatment for a number of hours, preferably from 4 to 16, at about 450° centigrade to 560° centigrade followed by an artificial aging for a number of hours, preferably from about 4 to 24, below 200° centigrade and preferably between about 150° centigrade to 200° centigrade. Increase in aging time usually results in increase in yield point and hardness.

In the specification and the appended claims, the term "magnesium base alloy" denotes an alloy containing more than 50 per cent magnesium, which metal may be either of high purity or may contain the usual impurities found in commercial magnesium.

I claim:

1. An alloy consisting of about 2 to 6 percent of zinc, about 4 to 8 per cent of tin, about 0.05 to 2 per cent of calcium, the balance being substantially magnesium.

2. An alloy consisting of about 0.1 to 20 per cent of tin, about 0.1 to 10 per cent of zinc, about 0.05 to about 2 per cent of calcium, the remainder being substantially magnesium.

3. An alloy consisting of about 0.1 per cent to 20 per cent of tin, about 0.1 per cent to 10 per cent of zinc, and about 0.05 per cent to 2.0 per cent of calcium the balance being substantially magnesium, characterized by high hardness and yield point and having an internal structure produced by a heat treatment of 4 to 16 hours at 450° centigrade to 560° centigrade followed by further aging treatment at a temperature less than 200° centigrade.

ROBERT T. WOOD.

115

120

125

130